

# UNITED STATES PATENT OFFICE.

GEORGE H. CHARLS, OF CANTON, OHIO.

## RUST-RESISTING ALLOY OF IRON.

1,355,589.

Specification of Letters Patent. Patented Oct. 12, 1920.

Application filed April 7, 1920. Serial No. 371,881.

No Drawing.

To all whom it may concern:

Be it known that I, GEORGE H. CHARLS, a citizen of the United States, and a resident of Canton, Stark county, State of Ohio, have invented an Improvement in 5 Rust-Resisting Alloy of Iron, of which the following is a specification.

This invention relates to rust-resisting alloys of iron. One of the objects thereof 10 is to provide a simple and practical alloy of iron having high rust-resisting qualities. Other objects are to provide metal of the above type which shall be inexpensive, shall require no especial heat treatment, and 15 which shall readily be formed into the desired shape. Other objects will be in part obvious and in part pointed out herein-after.

The invention accordingly consists in the 20 various features hereinafter set forth and more particularly defined in the following claims.

Considering now an illustrative embodiment of this invention, I propose to form 25 iron in any well known way, and wish to note at this point that I use the term "iron alloy" in a broad sense to cover alloys in which carbon may or may not be present, according as it is or is not specified. In 30 other words, the term "iron alloy" is to include compositions which might when the carbon content is present, be more specifically termed a steel alloy. It is also to be understood that in the alloys hereinafter 35 dealt with there are presumably present small amounts of phosphorus, sulfur, and other elements nearly always present in commercial iron and steel.

In the preferred embodiment of this invention, the carbon content is kept low, 40 preferably substantially below .20%. In fact, I have found that as the carbon is reduced throughout a considerable range below the above amount, the results are improved, 45 Even with the carbon eliminated, thus giving a simple iron compound, I have obtained excellent results.

A leading feature of this invention is the incorporation in the metal of a small 50 amount of the element molybdenum. For good results I prefer to keep the molybdenum content below .50% and much better results are gained with much smaller proportions of this alloy. In fact, the beneficial 55 effect increases as the molybdenum content is reduced and I have found excellent re-

sults with molybdenum present in a proportion of substantially .15%. The molybdenum however should not be reduced to an amount equal to the amount of sulfur 60 present.

The molybdenum is added preferably in the form of ferro-molybdenum and is added to the molten metal in the furnace, ladle or even in the ingot, and tends to distribute itself throughout the mass of the metal.

With ingots made in this manner, the rolling into sheets is readily accomplished or it may if desired be formed into wire or 70 other shapes, although especially advantageous results are gained with sheets. Such sheets are resistant to rust, or corrosion, to a high degree without special heat treatment or treatment of their surface.

As variations might be made in the above 75 illustrative embodiment of my invention or in the method by which it is made, it is to be understood that all matter herein set forth is to be interpreted as illustrative and not 80 in a limiting sense.

I claim as my invention:

1. A rust-resisting alloy of iron comprising in combination with the iron, a small amount of molybdenum, and not more than 85 .20% of carbon.

2. A rust-resisting alloy of iron comprising in combination with the iron, an amount of molybdenum less than .50% and less than .20% of carbon.

3. A rust-resisting alloy of iron comprising in combination with the iron, an amount of molybdenum less than .30% and less than .20% of carbon.

4. A rust-resisting alloy of iron comprising in combination with the iron, an amount of molybdenum less than .20% and less than .20% of carbon.

5. A rust-resisting alloy of iron comprising in combination with the iron, an amount of molybdenum less than .16% and less than .20% carbon.

6. A rust-resisting alloy of iron comprising in combination with the iron, an amount of molybdenum less than .16% and more 105 than the sulfur content, and carbon to an amount less than .20%.

7. A rust-resisting alloy of iron comprising in combination with the iron, a small amount of molybdenum, and less than .10% 110 of carbon.

8. A rust-resisting alloy of iron comprising

ing in combination with the iron, a small amount of molybdenum and less than .06% of carbon.

9. A rust-resisting alloy of iron comprising in combination with the iron, molybdenum to an amount less than .16%.

10. A rust-resisting alloy of iron comprising in combination with the iron, less

than .11% of carbon, and less than .16% of molybdenum, the molybdenum being in excess of the sulfur content.

In testimony whereof, I have signed my name to this specification this 3rd day of March, 1920.

GEORGE H. CHARLS.